

# UNITED STATES PATENT OFFICE.

PAUL FAEHR, OF BITTERFIELD, GERMANY, ASSIGNOR TO ELECTROCHEMISCHE WERKE,  
G. M. B. H., OF BERLIN, GERMANY.

## PYROPHORIC ALLOY.

1,102,575.

No Drawing.

Specification of Letters Patent.

Patented July 7, 1914.

Application filed March 27, 1912. Serial No. 686,667.

To all whom it may concern:

Be it known that I, PAUL FAEHR, a citizen of the United States, residing at 15 Bismarck street, Bitterfeld, Germany, have invented certain new and useful Improvements in Pyrophoric Alloys; and I do hereby declare the following to be a full, clear, and exact description of the invention, such as will enable others skilled in the art to which it appertains to make and use the same.

Recent investigations in the domain of pyrophoric rare-earth metal alloys have shown that for the production of commercially utilizable products it is by no means necessary to have a percentage of iron. Although Auer, in his Austrian Patent No. 19251, expressly insists that with the complete substitution of iron, the pyrophoric power is diminished in a way that cannot be disputed, this is by no means the case. Very good pyrophoric alloys can be obtained without an addition of iron, if zinc, cadmium, tin or lead is alloyed with cerium. Experiments to alloy zinc with cerium have heretofore been made (see Abegg's *Handbuch der Anorganischen Chemie*, 1906, vol. 111, part 1, page 195) but no sparking qualities whatever were observed in these alloys, and the described properties of the alloys in other respects were unfavorable to their commercial utilization.

The pyrophoric alloys hitherto known, which contain the "rare earth" metals are composed generally of single metals like: manganese, iron, nickel and cobalt and it would be entirely incorrect to suppose that all alloys of the rare earth metals possess pyrophoric properties. One must bear in mind that pyrophoric properties are by no means possessed, as a rule, by the cerium alloys, and must be regarded in fact in every respect as exceptional. The cerium copper alloy for instance has no pyrophoric properties whatever. In the periodic system copper is followed by zinc, and judging from the behavior of copper one would be led to suppose, that the zinc-alloy would also lack pyrophoric properties. It is therefore surprising that the zinc alloy should exhibit the favorable pyrophoric properties that it does. The elements directly following zinc in the periodic systems are out of the question for the production of pyrophoricity on account

of their outer properties. The next elements following are silver and cadmium. The silver-cerium alloy is not pyrophoric, and the favorable pyrophoric properties of the cadmium-cerium alloy used in this invention are therefore all the more surprising. In this connection it must be particularly taken into account that the cerium-cadmium alloy is altogether new. Hans Beck, who is the only one, who has investigated this subject, was unable to produce the cerium-cadmium alloys (Beck, *Beiträge zur Kenntnis der Metalle der Cer-Gruppe*, Nürnberg 1907, seite 27, absatz 2.) The properties of the cerium-cadmium alloys, which are described in this invention for the first time are likewise new and surprising. According to the publication of Beck even the possibility of the existence of a cerium-cadmium alloy must be regarded as a surprising fact.

I have now ascertained that alloys of the rare earth metals with zinc, cadmium, tin and lead, may be produced, which possess the appropriate hardness and brittleness, and which exhibit the property of sparking to an extraordinary degree when rubbed or scratched. The sparks of some of these alloys are of a higher brilliancy than those of pyrophoric alloys heretofore known. Furthermore, the sparks, especially of the cadmium-zinc-and tin rare-earth metal alloys are hotter than those of the cerium-iron alloys heretofore known, and furthermore, these new alloys are much more resistant to the air than the alloys heretofore known. The metals cadmium, lead, zinc and tin can be employed either singly or in admixture with each other, and cerium can be supplanted either entirely or partially by other rare earth metals. The production of the new alloys conforms simply to the procedure employed for the production of alloys in accordance with the usual working methods. It is advisable to add the metals in a careful manner to the melted cerium. When the cerium is melted in an electric furnace, it is likewise advisable not to undertake the mixing when the electric circuit is closed, as Auer proposes in the obtaining of his alloys. In the present instance, a large portion of the metals of addition would be volatilized, if this should

be permitted, or would be lost by passing off into the slag. If, however, the metals to be alloyed are mixed and carefully heated, we then obtain the desired alloys and without particular loss.

The proportions in which the zinc, cadmium, tin and lead are added to the molten rare earth metals, depend of course, entirely upon the desired degree of pyrophoricity, 10 the hardness and the other important technical qualities desired. The addition of the metals to the cerium has, among other things, the effect of increasing the hardness of the cerium aside from the diminution of the pyrophoric effect. The quantity of the addition is controlled by the circumstance that with larger additions the hardness increases. Too great hardness is to be avoided, as it increases the difficulty 20 of working the metal, and the difficulty of producing the sparks. Higher percentages of cadmium are permissible than of the other metals in making up the rare earth metal alloys in accordance with my invention.

By way of illustration, the composition of a few alloys that spark very well and that are economical in use are given below, although these form, so to speak, merely 30 samples of a multitude of possible combinations: 1. 40% cadmium with 60% cerium; 2. 30% zinc with 70% cerium; 3. 30% tin with 70% cerium; 4. 30% lead with 70% cerium. When two or more of the alloying 35 metals are added to the rare earth metal to form the desired alloy, the added metals may be in any appropriate proportions among themselves provided the aggregate of the additions represents the necessary 40 proportion with respect to the rare earth metal. For example, if 70% cerium be employed with the additional 30% consisting of a mixture of the other metals or any of them, the proportions of the individual 45 added metals may be varied as desired, an exemplary alloy being represented as follows: zinc 10%, tin 10%, lead 10%, cerium 70%. In order to modify the character of the sparks, additions of third metals, such as 50 magnesium, aluminium and calcium may be made. For certain purposes *e. g.*, for miners' lamps, too energetic an emission of sparks is not desirable; on the contrary, a compact flame is preferred. This property, 55 is inherent in alloys of given proportions only. In order to vary their hardness and their heating effect, it is desirable, therefore, to make use of the addition of third metals, as suggested.

60 The new alloys not only keep for an indefinite time when exposed to air but also in the presence of moisture neither are they affected by great changes of temperature nor by being placed in water. None of the 65 pyrophoric alloys hitherto known can fulfil

these conditions. The above mentioned properties are especially important for the ignition of miners' lamps. These lamps have to be used by the miners for a long time in moist warm places. Consequently 70 the safeness of the ignition becomes questionable, as soon as the alloys used for the purpose of ignition are acted on by moisture. Should this be the case the danger arises of not being able to ignite the lamps at all, or 75 even if the ignition is faulty and uncertain the safety of the miner can be imperiled.

The high temperature of combustion of the individual metal particles struck from the alloy must be especially emphasized as 80 this is of the greatest importance in respect to the ignition of safety lamps. For tiny metal particles can pass through the meshes of the gauze into the open air in spite of all precautions and can cause the greatest 85 disasters in any shaft not free from fire damp, if the particles have a low combustion temperature.

Experiments carried out by the mining 90 department have shown, that the unburned metal particles thrown off during the ignition can only be made to burn with the greatest difficulty on account of their high temperature of combustion and can never cause any explosion by a sudden accumulation 95 of fire damp. None of the alloys hitherto known have given such favorable results as the tests of the mining department. On account of their exceptional indifference to changes of temperature and the influence 100 of moisture the new alloys have a wide field of use in tropical countries, a fact that can not be asserted in regard to the known alloys.

The new alloys are particularly applicable 105 to the ignition of gaseous or liquid fuels, and also to the ignition of explosive mixtures. Their property of burning in a powdered condition with a high emission of heat and an intense radiation of light, makes 110 them appropriate to the production of igniting and illuminating devices of the most varied kinds.

The so-called "rare earth" metals are difficult to separate and consequently it is almost always necessary in practice to use a mixture of cerium with lanthanum and didymium, that is to say, a mixture of the metals of the cerium group of the "rare earth" metals.

Having thus described my invention, what I claim is:

1. A metal alloy containing a metal of the rare earth group and one or more of the metals, zinc, cadmium, tin, or lead in such 115 proportions as to make the alloy pyrophoric.

2. A metal alloy containing a metal of the rare earth group and one or more of the metals, zinc, cadmium, tin, or lead in such 125 proportions as to make the alloy pyrophoric,

with the addition of another metal for the purpose of modifying the character of the sparks.

3. A metal alloy containing cerium and 5 one or more of the metals, zinc, cadmium, tin, or lead in such proportions as to make the alloy pyrophoric.

4. A metal alloy containing cerium and 10 one or more of the metals, zinc, cadmium, tin, or lead in such proportions as to make the

alloy pyrophoric, with the addition of another metal for the purpose of modifying the character of the sparks.

In testimony whereof I affix my signature, in presence of two witnesses.

PAUL FAEHR.

Witnesses:

JULIUS RUINLAND,  
KARL BRIEKEBEN.